

Patented June 23, 1942

2,287,028

# UNITED STATES PATENT OFFICE

2,287,028

## MANUFACTURE OF ARTIFICIAL SPINNABLE MATERIAL

Angelo D'Ambrosio and Arnaldo Corbellini,  
Milan, Italy

No Drawing. Application March 9, 1938, Serial  
No. 194,934. In Italy November 26, 1936

16 Claims. (CL. 106—127)

This invention relates to the manufacture of artificial material by coagulation from mixed solutions of protein and viscose and enables articles such as spinnable filaments to be made from such solutions whilst utilizing in part already existing plants for the manufacture of artificial cellulosic filaments.

It is known that for a number of years attempts have been made to produce artificial spinnable material containing some protein substances and possessing wool- or silk-like properties. It is well known, however, that the materials of this character so far produced have not given satisfactory results due to their deficient mechanical and chemical properties and their high cost.

Among the cheapest protein materials the keratinous substances such as constitute horn, hooves, nails, and hair, and other proteins such as gluten, ossein and the like, which are insoluble in dilute alkali, have been considered and have attracted the attention of many investigators. The substances of the first of said groups have in particular been considered because they assimilate the properties of wool.

The said protein substances were dissolved in different solvents, having generally an alkaline or acid character, but the results were always unsatisfactory, mainly because the filaments obtained from these solutions did not possess sufficient strength or did not meet the requirements of practical utilization.

A difficulty arising in connection with proteins insoluble in dilute alkali is that the use of strong alkali causes decomposition of the protein. Thus according to the process described in the British specification No. 55,623 of 1925 the keratin, fibroin or the like is or are dissolved by means of caustic alkali and cellulose and carbon disulphide are added. By this process, because caustic alkali is employed, the molecules of the protein substance are subject to a strong decomposition, which is much more substantial than when sodium sulphide is employed as solvent, as recently proposed and which acts mainly as reducing and not as hydrolyzing agent.

In an article by Dr. Grawe published in the journal "Angewandte Chemie" No. 20, dated May 16, 1936, on page 306, it is stated that it is impossible to obtain a viscous solution of keratin by dissolving completely wool fibres in sodium sulphide. In this article it is stated: "By the action of 50 gms. of crystallized sodium sulphide and 115 gms. water on 100 gms. wool a viscous mass is obtained which still contains numerous undis-

solved fibers. In order to promote an action as uniform as possible it was necessary to mix thoroughly and repeatedly or to knead by means of apparatus and subsequently to work up the mass by means of a ball-mill. In order to obtain a homogeneous protein solution it is necessary to separate the dissolved from the undissolved keratin."

Due to the viscosity and the high degree of swelling of the undissolved parts in such a case, all known methods of filtration fall short. Filtration is only possible by packing the mass in a press filter cloth and compressing same in a cylinder closed at one side, an exactly fitting piston being pressed against the mass by means of a screw press. Having tried to produce artificial filaments from the keratin solution thus obtained, it was stated that, even when it was possible to spin the dissolved keratin, rough fibers were obtained which "show a very low strength when still wet and a very low elasticity after drying."

An object of this invention is an improved process of producing a solution of viscose and protein for the manufacture of artificial materials by coagulation, the said process being of particular advantage where the source of the protein is a material insoluble in dilute alkali, such as keratinous materials presenting the difficulties described in the article already referred to, gluten and ossein.

Further objects of the invention relate to the subsequent steps involved in obtaining an artificial material such as a filament from such a solution.

We have found that a satisfactory viscose-protein solution for the manufacture of artificial materials can be obtained, with proteins insoluble in dilute alkali by preparing in a known manner a paste of the keratin or other protein, and an alkaline sulphide, by homogenizing the same thoroughly and by leaving this paste for a sufficiently long time at a temperature of 15°—30° C., in order to obtain a practically complete protein liquor with the slightest possible decomposition of the protein molecules. By a suitably longer kneading operation, the maturing treatment at 15°—30° may be suitably shortened or even eliminated. The keratin or other protein liquor thus obtained cannot be filtered alone, but when mixed with a viscose solution already mature for spinning it constitutes together with this latter a mixed solution which unexpectedly is practically free from undissolved keratin parts and can be easily filtered and spun.

The protein liquor which can be mixed in any

suitable proportion with a viscose solution, thus forming viscous mixed solution, is prepared as follows:

The protein material insoluble in dilute alkali (for example, horn, hooves, nails, hair, or wool waste), is milled into a fine powder. This powder is treated in suitable kneaders and mixers with a solution containing 5-15 per cent of sodium sulphide. Depending on the kind of raw materials employed, for each 100 parts of protein material to be dissolved, 150-300 parts of this sulphide solution are usually employed. The viscous paste obtained by kneading and mixing the powdered protein with the solution of sodium sulphide is allowed to become fluid at a temperature of 15-30° C. for about 1 to 15 hours, according to the more or less thorough mechanical mixing and kneading and to the temperature employed, in which time it becomes substantially homogeneous. After this time a nearly complete dull-green liquor is obtained.

The keratin thus rendered fluid is thoroughly mixed with a viscose solution, for example cellulose xanthogenate, already mature for spinning, in which it is completely dissolved. This mixed solution can be rapidly filtered through the usual filter presses whereas the original keratin liquor was practically unfilterable. The mixing with cellulose xanthogenate can be effected in any proportion and it is practically possible to obtain mixed filaments or other articles having a protein content of say 90 per cent and more.

For convenience the application of the invention to the production and spinning of filaments will be considered.

Before spinning, the mixed solution obtained according to the invention is deaerated or degassed under vacuum in the usual manner.

Our spinning and coagulation is effected exactly as in the case of viscose silk.

The next step is the rendering insoluble or tanning of the filaments, which is effected as follows:

The filaments are first washed thoroughly with water in order to eliminate the acid coagulating liquor and are treated with a tanning liquid consisting preferably of an aqueous solution containing about 8 per cent of formic aldehyde with the addition of 4-6 per cent of alum and some lactic acid, and the whole is heated for a short time to 45-50° and then allowed to cool at room temperature, until the reaction is completed.

It is possible also to effect all the tanning at room temperature, or also to heat the tanning liquid in the last phase of the reactions. According to the procedure adopted the filaments show different characteristics.

It is also possible to avoid the employment of the organic acid if the filaments are not thoroughly washed after coagulation.

Particular advantageous characteristics are imparted to the filaments if same are dried after the tanning at a temperature of approximately 100-105° C.

In the before mentioned article it is stated, on page 303, that the subsequent treatment of the coagulated albuminoids with tanning reagents makes the filaments very rough. Now, by tanning the filaments in the manner as just described, this does not happen.

From the foregoing it will be apparent that the process just described permits of obtaining filaments and so forth having a protein content in simulation of wool whilst employing inexpen-

sive materials, especially those of the character indicated which are insoluble in weak alkali and from which it has not hitherto been thought possible to produce a solution capable of being filtered.

It is to be understood that the process just described is given only by way of example and can undergo numerous changes without departing from the spirit of the invention; thus, for instance, other additions to the sulphide solution can be made, and furthermore, as constituents of the tanning solution, instead of formic aldehyde other similarly acting reagents as acetic aldehyde, acrolein, furfural and the like can be employed, and instead of alum, aluminium sulphate or the like.

Likewise it is possible to precipitate, within or on the mixed filaments produced according to the invention, suitable insoluble, protecting or tarnishing or like substances in like manner as with artificial cellulose silk.

We claim:

1. The process of preparing a mixed solution of keratin and viscose for the manufacture of artificial material by coagulation, which comprises treating a keratinous material, in a finely powdered state, with an alkali sulphide solution, converting the mass to a fluid condition by a treatment which includes thorough mixing and mechanical kneading, and thereafter mixing the fluid mass with a viscose solution.

2. The process of preparing a mixed solution of keratin and viscose for the manufacture of artificial material by coagulation, which comprises treating a keratinous material, in a finely powdered state, with an alkali sulphide solution, converting the mass to a fluid condition by a treatment which includes thorough mixing and mechanical kneading, thereafter mixing the fluid mass with a viscose solution, and filtering the resultant solution.

3. The process of preparing a mixed solution of keratin and viscose for the manufacture of artificial material by coagulation, which comprises thoroughly mixing and mechanically kneading a keratinous material, in a finely powdered state, with an alkali sulphide solution, maturing the mass at temperatures within the range 15 to 30° C. to attain a fluid condition thereof, thereafter mixing the fluid mass with a viscose solution, and filtering the resultant solution.

4. The process of preparing a mixed solution of keratin and viscose for the manufacture of artificial material by coagulation, which comprises thoroughly mixing and mechanically kneading a keratinous material, in a finely powdered state, with an alkali sulphide solution in the proportion of 100 parts of keratinous material to 150 to 300 parts of a 5 to 15% aqueous solution of an alkali sulphide, causing the mass to attain a fluid condition, thereafter mixing the fluid mass with a viscose solution, and filtering the resultant solution.

5. The process of preparing a mixed solution of keratin and viscose for the manufacture of artificial material by coagulation, which comprises thoroughly mixing and mechanically kneading a keratinous material, in a finely powdered state, with an alkali sulphide solution, in the proportion of 100 parts of keratinous material to 150 to 300 parts of a 5 to 15% aqueous solution of an alkali sulphide, maturing the mass at temperatures within the range of 15 to 30° C. to attain a fluid condition thereof, thereafter mixing the

fluid mass with a viscose solution, and filtering the resultant solution.

6. The process of preparing a mixed solution of keratin and viscose for the manufacture of artificial material by coagulation, which comprises treating a keratinous material insoluble in weak alkali, in a finely powdered state, with an alkali sulphide solution, converting the mass to a fluid condition by a treatment which includes thorough mixing and mechanical kneading, and thereafter mixing the fluid mass with a viscose solution.

7. The process of preparing a mixed solution of keratin and viscose for the manufacture of artificial material by coagulation, which comprises thoroughly mixing and mechanically kneading a keratinous material insoluble in weak alkali, in a finely powdered state, with an alkali sulphide solution, maturing the mass at temperatures within the range 15 to 30° C. to attain a fluid condition thereof, thereafter mixing the fluid mass with a viscose solution, and filtering the resultant solution.

8. The process of preparing a mixed solution of keratin and viscose for the manufacture of artificial material by coagulation, which comprises thoroughly mixing and mechanically kneading a keratinous material insoluble in weak alkali, in a finely powdered state, with an alkali sulphide solution in the proportion of 100 parts of keratinous material to 150 to 300 parts of a 5 to 15% aqueous solution of an alkali sulphide, maturing the mass at temperatures within the range 15 to 30° C. to attain a fluid condition thereof, thereafter mixing the fluid mass with a viscose solution, and filtering the resultant solution.

9. A process of manufacturing artificial materials, comprising in combination the steps of preparing a keratin viscose solution in the manner claimed in claim 6, thereafter degassing the solution and coagulating the same in a wet coagulation bath, and subsequently tanning the coagulated material in a bath containing a keratin insolubilizing agent, a water soluble aluminium salt, and a weak organic acid, the tanning being effected in part at room temperature and in part at temperatures of 45 to 50° C., and the tanned filaments being washed and then dried at a temperature under 100° C.

10. A process of manufacturing artificial materials, comprising in combination the steps of preparing a keratin viscose solution in the manner claimed in claim 6, thereafter degassing the solution and coagulating the same in a wet coagulation bath, and subsequently tanning the coagulated material in a bath containing about 8% of a keratin coagulating aldehyde, 4 to 6% of alum, and a weak acid, washing the material with water and then drying first at a temperature under 100° C. and finally at a temperature of 100 to 105° C.

11. A process of manufacturing artificial materials, comprising in combination the steps of preparing a keratin viscose solution in the man-

ner claimed in claim 6, thereafter degassing the solution and coagulating the same in a wet coagulation bath, and subsequently tanning the coagulated material in a bath containing a keratin insolubilising agent, a water soluble aluminium salt, and a weak organic acid, and washing the material with water and then drying first at a temperature under 100° C. and finally at a temperature of 100 to 105° C.

12. A process of manufacturing artificial materials, comprising in combination the steps of preparing a keratin viscose solution in the manner claimed in claim 6, thereafter degassing the solution and coagulating the same in a wet coagulation bath, and subsequently tanning the coagulated material in a bath containing a keratin insolubilising agent, a water soluble aluminium salt, and a weak organic acid, the tanning being effected by first treating the material in the tanning bath then raising the tanning bath to a temperature of 45 to 50° C., and then allowing the bath to cool slowly, the filaments being left in the bath at room temperature until the tanning is complete.

13. The process of preparing a mixed solution of keratin and viscose for the manufacture of artificial material by coagulation which comprises treating a keratinous material, in a finely powdered state, with a sodium sulphide solution, converting the mass to a fluid condition by a treatment which includes thorough mixing and mechanical kneading, and thereafter mixing the fluid mass with a viscose solution.

14. The process of preparing a mixed solution of keratin and viscose for the manufacture of artificial material by coagulation, which comprises treating a keratinous material, in a finely powdered state, with a sodium sulphide solution, converting the mass to a fluid condition by a treatment which includes thorough mixing and mechanical kneading, thereafter mixing the fluid mass with a viscose solution, and filtering the resultant solution.

15. The process of preparing a mixed solution of keratin and viscose for the manufacture of artificial material by coagulation, which comprises treating a keratinous material insoluble in weak alkali, in a finely powdered state, with a sodium sulphide solution, converting the mass to a fluid condition by a treatment which includes thorough mixing and mechanical kneading, and thereafter mixing the fluid mass with a viscose solution.

16. The process of preparing a mixed solution of keratin and viscose for the manufacture of artificial material by coagulation, which comprises thoroughly mixing and mechanically kneading a keratinous material insoluble in weak alkali, in a finely powdered state, with a sodium sulphide solution, maturing the mass to attain a fluid condition thereof, thereafter mixing the mass with a viscose solution, and filtering the fluid resultant solution.

ANGELO D'AMBROSIO.  
ARNALDO CORBELLINI.